

July 19, 1966

K. P. BELLINGER

3,261,733

METHOD OF DISSOLVING A PLUG FROM A BIMETALLIC  
METAL CORE AND ETCHING BATH

Filed July 2, 1963



INVENTOR  
KENNETH P. BELLINGER

BY

*Peter L. Costas*

ATTORNEY

## 1

3,261,733

**METHOD OF DISSOLVING A PLUG FROM A BI-METALLIC METAL CORE AND ETCHING BATH**  
Kenneth P. Bellinger, Ellington, Conn., assignor to Conversion Chemical Corporation, Rockville, Conn., a corporation of ConnecticutFiled July 2, 1963, Ser. No. 292,325  
6 Claims. (Cl. 156—3)

The present invention relates to metal fabrication and more particularly to a novel bath and method for removing cores of iron, molybdenum and copper from initial assemblies with other metals.

This application is a continuation-in-part of copending application Serial Number 254,426, filed January 28, 1963, now abandoned.

In the fabrication of various metals such as titanium, zirconium, tungsten, aluminum and their alloys, it is often desirable to employ a core of another metal about which the primary metal is formed. For example, in forming nuclear reactor cores, plugs of iron or copper may be employed to define the desired apertures and titanium or zirconium is formed therearound. Subsequently, the core is dissolved in a bath of nitric acid. In forming filaments for light bulbs, tungsten wire is wound around an iron or molybdenum core and set; thereafter, the core is dissolved in a bath of nitric acid. Generally, such core-removing operations are characterized by a very high degree of exothermic activity, extremely rapid metal removal and copious fuming. The highly exothermic and rapid reaction has created serious problems in control of the operation, and fumes evolved by the operation have presented most significant problems from industrial hygiene and anti-pollution standpoints. Various scrubbers and treatments have been proposed and utilized at great expense and without complete efficacy in an effort to cope with the problem.

The term "core" as used herein refers to inserts, mandrels and various shapes of dissolvable metals selected from the group consisting of iron, copper and molybdenum which are readily dissolved by nitric acid baths. Generally, low carbon iron or cold-rolled low carbon steel of low alloy content are the preferred ferrous materials to avoid contamination by alloying elements. Similarly, copper and molybdenum should be of low alloy content.

It is an object of the present invention to provide a novel bath for removing metal cores from initial assemblies with other metals formed thereabout and substantially inert to the bath which bath is characterized by rapid but relatively controlled action and substantially freedom from fuming.

Another object is to provide a method for removing metal cores from initial assemblies with other metals which is rapid, relatively controlled and substantially free from fuming.

Other objects and advantages will be readily apparent from the following detailed specification and claims and the attached drawing wherein:

FIGURE 1 is a diagrammatic illustration of apparatus in which a process embodying the present invention is being conducted.

It has now been found that the foregoing and related objects may be readily attained by forming about a dissolvable core of a metal selected from the group consisting of iron, molybdenum and copper a primary metal to produce an initial assembly; and thereafter immersing the initial assembly in a core-removing bath for a period of time sufficient to dissolve the core, the core-removing bath comprising an aqueous solution consisting essentially of 15.0 to 42.0 percent by weight nitric acid, 2.0 to 28.0 percent by weight of a reaction-controlling agent selected from the group consisting of urea and melamine, and 40.0 to 80.0 percent by weight water. In operation, the

## 2

bath should develop a foam blanket for optimum effectiveness in eliminating nitric oxide fumes, but excessive frothing should be avoided to maintain effective core-dissolving action as by a cooling grid above the bath or by ultrasonic energy. This method has significant advantages in the forming of tungsten, zirconium, titanium and aluminum since it effects the speedy removal of the core in a relatively controllable reaction while being substantially innocuous to the formed primary metal thereabout.

The molar ratio of reaction-controlling agent to nitric acid is about 0.1 to 0.75:1, and preferably about 0.25 to 0.60:1 for iron and molybdenum cores and about 0.15 to 0.45:1 for copper cores. When the nitric acid is in the range of about 35.0 to 42.0 percent by weight of the bath and/or when the iron or molybdenum core metal present in the bath is sufficient to expend substantially the nitric acid, it is generally necessary to use a molar ratio of about 0.3 to 0.6:1 to eliminate fuming and maintain the reaction under control. When treating copper cores, it is generally necessary to use lower weight percentages and molar ratios of reaction-controlling agent since it appears to produce or favor the formation of a barrier coating on the copper core which limits the attack of the nitric acid. Use of the higher molar ratios of reaction-controlling agents may produce a significant increase in viscosity and/or the development of a pasty condition due to the formation of a precipitate requiring control of the frothing and/or increase in temperature.

The bath temperature should be maintained in the range of about 140 to 210° Fahrenheit, and most desirably about 170 to 200° Fahrenheit. When more than about 10 percent by weight of reaction-controlling agent is used, it is generally necessary to maintain a temperature of about 180 to 200° Fahrenheit to dissolve the agent and to reduce excessive viscosity in the bath. Temperatures of about 170 to 200° Fahrenheit are desirable for maintaining optimum effectiveness of the bath in removing copper cores. Although the bath generates heat during treatment, generally it is necessary to heat the bath initially to obtain full solution of or dispersion of the higher weight percentages of urea. Particularly when the bath volume is small or when continuing use is being conducted with iron or molybdenum cores, cooling coils may be desirably provided to prevent the bath from overheating due to the exothermic reaction and from possibly reaching the boiling point or from developing excessive froth.

The method of the present invention is rapid and highly exothermic but can provide greater control than a conventional nitric acid bath while eliminating substantially the evolution of nitric oxide. Since the reaction is controlled, nitric acid spray is reduced, and the hazards to the operator are minimized. Removal of as much as one-third of an iron core within a minute in assemblies presenting relatively large surface area is possible with the preferred bath composition operating at the preferred temperature range. Thus, rack treatment of assemblies is possible with the time of immersion required being readily determinable by preliminarily treating a test assembly and visually determining the time required for complete removal of the iron core in the remaining assemblies. Moreover, it has been found that the nitric oxide fuming may be reduced from in excess of 300,000 parts per million to 300 parts per million, and even less. In this manner, high rates of production may be maintained at elevated bath temperatures without expensive fume-scrubbing installations.

The preferred baths of the present invention for iron and molybdenum cores consist essentially of about 28.0 to 38.0 percent by weight nitric acid, 47.0 to 54.0 percent by weight water and 8.0 to 20.0 percent by weight of the reaction-controlling agent with a molar ratio of reaction-controlling agent to nitric acid of about 0.2 to 0.6:1, and

most desirably of about 0.35 to 0.55:1. For copper cores, the bath preferably contains only about 4.0 to 10.0 percent of reaction-controlling agent with a molar ratio of about 0.15 to 0.45:1.

Although melamine may be used alone to provide the lower molar ratios and with urea in combination, urea has been found far more preferable because of optimum operating characteristics, cost, lower molecular weight and greater solubility to provide the more effective higher molar ratios.

Although the urea may be added in increments during the operation of the bath, this technique provides a less effective bath and presents substantial hazards since a relatively strong reaction takes place when urea is added to a hot nitric acid solution. Lesser amounts of urea may be used with incremental addition of further amounts with some loss in effectiveness when a plurality of cycles will be run in a given bath and the urea is added slowly between cycles. The bath is preferably formulated by first dissolving the urea in hot water because of its limited solubility.

The method of the present invention is rapid and highly exothermic but can provide greater control than a conventional nitric acid bath while eliminating substantially the evolution of nitric oxide fumes. The baths of the present invention function efficiently even when the surface of the metal has an oxide scale and appear to enhance the action of the nitric acid on some cores. By achieving control of the rate of the reaction, the excessive frothing produced by gas bubbles within the bath can be reduced so that the bath can function more efficiently.

Although the mechanism of the present invention is not fully understood, it is believed that the urea cooperates with the nitric acid within the above-described compositional limits at temperatures above 140° Fahrenheit by modifying the reaction taking place at the bath-core interface. The rate of metal attack rises rapidly with increase in temperature to about 210° Fahrenheit and the solubility of urea increases (or the viscosity of the mixture decreases) to permit increase in its beneficial action. In contrast with conventional baths which have a deep brown color after contact with the core, the baths of the present invention generally retain a greenish hue and, in place of a heavy froth, generally have a blanket of foam over the top of the bath. This foam presumably presents a large surface area of urea in the foam wall acting to increase the likelihood of reaction with fumes escaping from the body of the bath. The foam layer initially increases in depth with increase in urea concentration and also appears to increase in viscosity to a point of relatively highly concentration after which the foam layer seems to stabilize or decrease in depth.

Although passing fumes evolved from the nitric acid bath through a scrubbing solution containing urea in about 4.0 to 30.0 percent by weight will produce substantial conversion of nitric oxide fumes, generally substantially complete elimination in the treatment tank is desirable to ensure efficacy of the bath operation and control and to minimize health hazards resulting from possible defects in the exhaust or scrubbing systems. With the core-dissolving baths of the present invention, scrubbing the fume in water alone or water with some alkali is sufficient to remove the nitric acid fumes and any trace amounts of other noxious gases such as nitrogen dioxide since the predominant nitric oxide is apparently converted to nitrogen within the bath and its foam blanket, analyses 15 indicating the presence of nitrogen and carbon dioxide.

The initial assembly should be completely immersed within the bath and be covered by more than four, and desirably more than six, inches of bath. In practice, the deeper is the immersion, the more efficient is the fume 20 removal. The assemblies can be racked or individually lowered into the bath.

Referring now to the attached drawing, therein diagrammatically shown is a process embodying the present invention. The work tank 2 contains the bath 4 in which 25 is immersed the initial assembly generally designated by the numeral 6 and having a core 8 of a dissolvable metal with the primary metal 10 formed thereabout. As illustrated, the assembly 6 is disposed well below the surface of the bath 4 which has a foam blanket 12 of substantial depth thereover. Any fumes and spray evolving from the bath 4 are entrapped in the hood 14 and carried by the conduit 16 to the bottom of the scrubber tank 18 so that they are washed thereby prior to being discharged to the atmosphere by the conduit 20. As hereinbefore 30 stated, the scrubber may use water alone, water containing urea, or water containing alkali to neutralize nitric acid fumes.

Illustrative of the effect of varying the molar ratio (and weight percentage) of urea in a bath containing 40 50.0 percent by volume of nitric acid (42° Baumé) and 50.0 percent by volume of water is Table 1. In the tests reported in Table 1, ferrous specimens were immersed in 200 cc. of the bath in a 500 cc. graduate for one hour, 45 the bath having been preheated to the indicated temperature. The ferrous specimens in these tests are plural pieces of wire of 0.196 inch diameter and about 0.25 inch cut on a diagonal. The wire was of 1013 alloy nominally composed of 0.14 percent by weight carbon, 0.65 percent 50 by weight manganese with the remainder substantially iron with sulfur and phosphorus impurities. The presence or absence of brown nitric oxide fumes above the bath in the graduate and weight loss are noted as evidencing the efficacy of the baths of the invention.

TABLE 1

| HNO <sub>3</sub> ,<br>Percent<br>by wt. | H <sub>2</sub> O,<br>Percent<br>by wt. | Urea,<br>Percent<br>by wt. | Molar<br>Ratio<br>Urea:<br>HNO <sub>3</sub> | Steel,<br>Grams | Tempera-<br>ture,<br>Degrees<br>F. | Time for Main Re-<br>action to Subside<br>or Steel to Dis-<br>solve, Minutes | Fuming                                             | Wt.<br>Loss,<br>Grams |
|-----------------------------------------|----------------------------------------|----------------------------|---------------------------------------------|-----------------|------------------------------------|------------------------------------------------------------------------------|----------------------------------------------------|-----------------------|
| 39.2                                    | 60.1                                   | 0.7                        | 0.02:1                                      | 20              | 180                                | 20                                                                           | Heavy                                              | 17.                   |
| 39.2                                    | 60.1                                   | 0.7                        | 0.02:1                                      | 4               | 180                                | 10 (consumed)                                                                | do                                                 | Total.                |
| 39.0                                    | 59.8                                   | 1.2                        | 0.04:1                                      | 20              | 180                                | 30                                                                           | do                                                 | 17.                   |
| 39.0                                    | 59.8                                   | 1.2                        | 0.04:1                                      | 4               | 180                                | 10 (consumed)                                                                | do                                                 | Total.                |
| 38.7                                    | 59.1                                   | 2.2                        | 0.06:1                                      | 20              | 180                                | 30                                                                           | do                                                 | 16.5.                 |
| 38.7                                    | 59.1                                   | 2.2                        | 0.06:1                                      | 4               | 180                                | 6 (consumed)                                                                 | do                                                 | Total.                |
| 37.8                                    | 57.8                                   | 4.4                        | 0.13:1                                      | 20              | 180                                | 60 <sup>1</sup>                                                              | do                                                 | 15.3.                 |
| 37.8                                    | 57.8                                   | 4.4                        | 0.13:1                                      | 4               | 180                                | 10 (consumed)                                                                | Heavy 3 min., diminished to light or none.         | Total.                |
| 36.3                                    | 55.3                                   | 8.4                        | 0.25:1                                      | 20              | 180                                | 40                                                                           | Heavy 5 min., diminished to medium, then to light. | 16.4.                 |
| 36.3                                    | 55.3                                   | 8.4                        | 0.25:1                                      | 4               | 180                                | 10 (consumed)                                                                | Medium, diminishing to light                       | Total.                |
| 35.0                                    | 53.6                                   | 11.4                       | 0.35:1                                      | 20              | 180                                | 50                                                                           | after 1 minute.                                    | 17.3.                 |
| 35.0                                    | 53.6                                   | 11.4                       | 0.35:1                                      | 4               | 180                                | 8 (consumed)                                                                 | Slight for 30 seconds.                             | Total.                |
| 33.6                                    | 51.6                                   | 14.8                       | 0.50:1                                      | 20              | 190                                | 50                                                                           | do                                                 | 17.0.                 |
| 33.6                                    | 51.6                                   | 14.8                       | 0.50:1                                      | 4               | 190                                | 10 (consumed)                                                                | Heavy                                              | Total.                |
| 39.5                                    | 60.5                                   | -----                      | -----                                       | 20              | 180                                | 12 (consumed)                                                                | do                                                 | 19.0.                 |

<sup>1</sup> Frothed out of graduate.

As will be readily appreciated, the ferrous wire specimens in the tests reported in Table 1 presented a large surface area to the bath for purposes of establishing severe conditions. In the following Table 2, tests using as the specimens a single slug of the ferrous alloy under similar conditions are set forth to show the effect of reduction in surface area.

Illustrative of the efficacy of the present invention are the following specific examples:

A bath was prepared by admixing 100 cc. of nitric acid (42° Baumé) and 100 cc. of water. A slug of low car-

TABLE 2

| HNO <sub>3</sub> , Percent by wt. | H <sub>2</sub> O, Percent by wt. | Urea, Percent by wt. | Molar Ratio Urea: HNO <sub>3</sub> | Steel, Grams | Temperature, Degrees F. | Time for Main Reaction to Subside or Steel to Dissolve, Minutes | Fuming                  | Wt. Loss, Grams |
|-----------------------------------|----------------------------------|----------------------|------------------------------------|--------------|-------------------------|-----------------------------------------------------------------|-------------------------|-----------------|
| 39.5                              | 60.5                             | 2.2                  | 0.06:1                             | 25.3         | 180                     | 15                                                              | Heavy -----             | 17.9            |
| 38.7                              | 59.1                             | 2.2                  | 0.06:1                             | 25.3         | 180                     | 15                                                              | do -----                | 17.8            |
| 35.0                              | 53.6                             | 11.4                 | 0.35:1                             | 25.3         | 185                     | 15                                                              | Medium for about 5 min. | 15.5            |
| 34.5                              | 52.7                             | 12.8                 | 0.42:1                             | 25.3         | 185                     | 20                                                              | Light for about 2 min.  | 16.3            |
| 33.6                              | 51.6                             | 14.8                 | 0.50:1                             | 26.1         | 190                     | 25                                                              | do -----                | 16.1            |

<sup>1</sup> Froth spilled out of graduate.

In Table 3 are set forth the results of similar tests on copper using as specimens pieces of #12 gauge wire to present a relatively high surface area.

bon steel (No. 1013, containing 0.14 percent by weight carbon and 0.65 percent by weight manganese) weighing 25.3 grams was immersed in the bath which had been

TABLE 3

| HNO <sub>3</sub> , percent by wt. | H <sub>2</sub> O, percent by wt. | Urea, percent by wt. | Molar Ratio Urea: HNO <sub>3</sub> | Cu, G. | Temp., °F. | Fuming        | Wt. Loss, Grams   |
|-----------------------------------|----------------------------------|----------------------|------------------------------------|--------|------------|---------------|-------------------|
| 39.2                              | 60.1                             | 0.7                  | 0.02:1                             | 33     | 180        | Heavy -----   | <sup>1</sup> 18.8 |
| 39.0                              | 59.8                             | 1.2                  | 0.04:1                             | 33     | 180        | do -----      | <sup>1</sup> 18.3 |
| 38.7                              | 59.1                             | 2.2                  | 0.06:1                             | 33     | 180        | do -----      | 1 25.0            |
| 37.8                              | 57.8                             | 4.4                  | 0.13:1                             | 33     | 180        | Medium -----  | <sup>2</sup> 17.9 |
| 37.8                              | 57.8                             | 4.4                  | 0.13:1                             | 11     | 180        | Light, 5 min. | Total             |
| 36.3                              | 55.3                             | 8.4                  | 0.25:1                             | 33     | 180        | Med., 2 min.  | 15.2              |
| 35.0                              | 53.6                             | 11.4                 | 0.35:1                             | 33     | 180        | None -----    | <sup>3</sup> 7.5  |
| 39.5                              | 60.5                             | -----                | -----                              | 33     | 180        | Heavy -----   | 29.6              |
| 35.0                              | 53.6                             | 11.4                 | 0.35:1                             | 33     | 190        | None -----    | <sup>4</sup> 9.0  |

<sup>1</sup> Spilled out of graduate badly.

<sup>2</sup> Spilled out to small amount.

<sup>3</sup> Green crystals formed in graduate during reaction and copper became coated.

<sup>4</sup> Heat continuously applied.

Illustrative of the several variables of the bath of the present invention on activity are the data set forth in Table 4. Test specimens of SAE 1010 cold-rolled steel 1 inch x 1.5 inches x 0.030 inch and weighing 5 grams were suspended in aqueous baths of the indicated composition at the temperatures and times indicated. Within the preferred range of bath composition, even initial fuming during the short period of immersion was eliminated. It will be noted that amounts of nitric acid or urea in excess of the aforescribed compositional limits greatly affected the activity.

placed in a 500 cc. graduate and preheated to 180° Fahrenheit. The reaction was accompanied by violent pumping and agitation with a froth reaching nearly to the top of the cylinder. Extremely copious brown fumes rose from the bath which had a dark brown color. After about fifteen minutes, the reaction subsided appreciably and after one hour the weight loss was found to be 17.9 grams.

TABLE 4

| HNO <sub>3</sub> , percent by wt. | H <sub>2</sub> O, percent by wt. | Urea, percent by wt. | Temp. Increase, °F. | Time, Sec. | Weight Loss, percent | Fuming       |
|-----------------------------------|----------------------------------|----------------------|---------------------|------------|----------------------|--------------|
| 1 49.5                            | 24.2                             | 26.3                 | 160-180             | -----      | Paste                | Paste.       |
| 1 42.3                            | 35.4                             | 22.3                 | 160-180             | 13         | 8                    | Heavy.       |
| 1 42.3                            | 35.4                             | 22.3                 | 180-200             | 16         | 14                   | Do.          |
| 1 44.3                            | 44.0                             | 11.7                 | 160-180             | 12         | 18                   | Do.          |
| 1 39.7                            | 39.5                             | 20.8                 | 160-180             | 15         | 15                   | Do.          |
| 1 40.8                            | 48.5                             | 10.7                 | 160-180             | 12         | 9                    | Do.          |
| 36.8                              | 43.8                             | 19.4                 | 160-180             | 20         | 12                   | Moderate.    |
| 35.6                              | 42.5                             | 21.9                 | 180-190             | 60         | 13                   | Very slight. |
| 38.2                              | 51.7                             | 10.1                 | 160-180             | 10         | 14                   | Heavy.       |
| 38.2                              | 51.7                             | 10.1                 | 180-200             | 18         | 18                   | Do.          |
| 34.8                              | 46.9                             | 18.3                 | 160-180             | 20         | 21                   | None.        |
| 34.8                              | 46.9                             | 18.3                 | 180-200             | 12         | 14                   | Do.          |
| 34.6                              | 41.1                             | 24.3                 | 180-190             | 60         | 12                   | Do.          |
| 32.6                              | 50.3                             | 17.1                 | 160-180             | 12         | 13                   | Do.          |
| 32.6                              | 50.3                             | 17.1                 | 180-200             | 18         | 27                   | Do.          |
| 19.3                              | 70.5                             | 10.2                 | 160-170             | 90         | 11                   | Very slight. |
| 19.3                              | 70.5                             | 10.2                 | 180-190             | 60         | 13                   | None.        |
| 16.8                              | 78.8                             | 4.4                  | 160-170             | 30         | 6                    | Do.          |
| 16.1                              | 75.5                             | 8.4                  | 160-170             | 30         | 8                    | Do.          |

<sup>1</sup> These formulations were very pasty even at elevated temperatures due to a precipitate.

A similar test was conducted with a bath additionally containing 42.0 grams of urea and heated to 190° Fahrenheit initially. In this instance, a foam blanket was generated which extended to about four inches from the top of the graduate. The bath retained a greenish hue throughout and only very light fuming occurred for the first two minutes during the development of the foam blanket and thereafter there was no evidence of fuming. The reaction subsided substantially after twenty-five minutes and, after one hour, the weight loss was determined at 16.1 grams.

*Example 2*

A bath was prepared by admixing 200 cc. of 42° Baumé nitric acid and 200 cc. water. A test specimen of SAE 1010 cold-rolled steel 1 inch x 4 inches x 0.030 inch and weighing 18 grams was immersed in the resultant bath at an initial temperature of 180° Fahrenheit. The specimen was withdrawn after the bath had reached a temperature of 200° Fahrenheit, a time period of about thirteen seconds. The test specimen was weighed and determined to have incurred a 26 percent weight loss. During the treatment operation, there was extremely copious fuming.

To a bath of the same composition was added 50 grams of urea and a similar test specimen was immersed therein at a temperature of 180° Fahrenheit and withdrawn after the bath temperature had reached 200° Fahrenheit, a time period of sixteen seconds. The test specimen was weighed and found to have incurred a 23 percent weight loss. During the treatment, there was but a slight evolution of fume.

Another bath was prepared by adding 100 grams urea, and the test was repeated. The time for the bath temperature to rise from 180 to 200° Fahrenheit was twenty-eight seconds, and the weight loss of the specimen was 29 percent. No fuming occurred during the treatment.

*Example 3*

A bath was prepared by admixing 500 cc. of 42° Baumé nitric acid, 500 cc. water and 125 grams melamine. A test specimen of cold-rolled steel weighing 18 grams was immersed in the bath at an initial temperature of 180° Fahrenheit and withdrawn therefrom after the bath had reached a temperature of 200° Fahrenheit, a time period of about forty seconds, during which there was extensive fume evolution.

The test was repeated with a bath containing 250 grams of melamine with the time period for the temperature to rise from 180 to 200° Fahrenheit being about fifty seconds. The treated specimen was weighed and found to have undergone a weight loss of 17.5 percent. During the period of immersion, there was but a very slight amount of fuming.

*Example 4*

Tungsten wire was wound about a core of molybdenum of variable diameter tapering to a point to form an initial assembly. The resulting assembly was immersed in a bath containing 50.0 percent by volume 42° Baumé nitric acid, 50.0 percent by volume water and 250 grams urea per liter and operated at a temperature of about 160 to 180° Fahrenheit.

The molybdenum core was dissolved out with substantially no fume evolution and the tungsten wire was not attacked.

*Example 5*

A nuclear reactor component was produced by forming Zircalloy (nominal composition—1.5 percent tin, 0.15 percent iron, 0.10 percent chromium, 0.05 percent nickel, and zirconium) about low carbon steel cores to define apertures therein.

The component was then immersed in a bath essentially the same as that in Example 4 and operated at a temperature of about 160 to 180° Fahrenheit. The steel cores were dissolved out with substantially no fume evolution.

*Example 6*

A bath was prepared by admixing 100 cc. of nitric acid (42° Baumé) and 100 cc. of water. Apparatus was provided to collect fumes evolved from the bath and wash them in a water scrubber provided by an Erlenmeyer flask. The bath was preheated to 180° Fahrenheit and a low carbon steel plug of 25.3 grams was placed therein. The reaction was violent and heavy brown fumes flowed from the bath and through the scrubber. After about twelve minutes, the reaction slowed appreciably and after one hour, the weight loss was found to be 17.9 grams.

A similar test was conducted using a bath additionally containing 22 grams of urea. Although the bath frothed, the reaction was less violent. Moderate fuming for the first five minutes diminishing to light was evident in the bath vessel, but little or no fumes were evolved from the water scrubber. After one hour, the weight loss was found to be 16.4 grams.

*Example 7*

A bath was formulated by admixing 75 cc. of nitric acid (42° Baumé), 75 cc. of water and 12.5 grams of urea. A specimen of molybdenum weighing 1.6 grams was completely dissolved in eighteen minutes in a rapid but controlled reaction. In a similar test bath containing no urea, heavy brown fumes were evolved.

*Example 8*

A bath was formulated containing 50 percent by volume nitric acid (42° Baumé) and 50 percent by volume water. To 300 cc. of this formulation which had been preheated to 180° Fahrenheit was added pieces of #12 gauge copper wire. Copious brown fumes were evolved and the reaction was violent.

A similar test was conducted with a bath additionally containing 24 grams of urea. Slight fuming occurred only initially. After one hour, 37.8 grams of copper was dissolved; after continuing immersion overnight, 39.8 grams was dissolved.

Thus, it can be seen that the method and bath of the present invention permit speedy but controlled removal of core metals of an initial assembly. Bath activity in some instances may be enhanced and in other instances is not extensively affected, but bath action is more controlled and fume evolution is substantially eliminated to reduce hygiene and fume-disposal problems.

Having thus described the invention, I claim:

1. The method of forming metals substantially inert to concentrated nitric acid comprising forming about a core of a dissolvable metal selected from the group consisting of iron, molybdenum and copper a primary metal substantially inert to nitric acid to produce an initial assembly; and immersing said initial assembly in a core-removing bath for a period of time sufficient to dissolve said core, said bath being at a temperature of about 140 to 210° Fahrenheit and comprising an aqueous solution consisting essentially of about 15.0 to 42.0 percent by weight nitric acid, 2.0 to 28.0 percent by weight of a reaction-controlling agent selected from the group consisting of urea and melamine, and 40.0 to 80.0 percent by weight water, said bath having a molar ratio of reaction-controlling agent to nitric acid of 0.1 to 0.75:1.0, the immersion of said initial assembly in said bath producing a blanket of foam on the top of said bath through which fumes must pass.

2. The method in accordance with claim 1 wherein said substantially inert metal is selected from the group consisting of titanium, zirconium, tungsten and alloys thereof.

3. The method of forming metals substantially inert to nitric acid comprising forming about a core of dissolvable metal selected from the group consisting of iron, molybdenum and copper a primary metal substantially inert to nitric acid to produce an initial assembly; and immersing said initial assembly in a core-removing bath for a period of time sufficient to dissolve said core, said bath having a temperature of about 180 to 200° Fahrenheit and com-

prising an aqueous solution consisting essentially of about 28.0 to 38.0 percent by weight nitric acid, 8.0 to 20.0 percent by weight of a reaction-controlling agent selected from the group consisting of urea and melamine, and 47.0 to 54.0 percent by weight water, the molar ratio of reaction-controlling agent to nitric acid being selected from the group consisting of (A) 0.35 to 0.55:1.0 when said dissolvable metal is selected from the group consisting of iron and molybdenum; and (B) 0.15 to 0.45:1.0 when said dissolvable metal is copper, the immersion of said initial assembly in said bath producing a blanket of foam on the top of said bath through which fumes must pass.

4. The method in accordance with claim 3 wherein said substantially inert metal is selected from the group consisting of titanium, zirconium, tungsten and alloys thereof.

5. The method in accordance with claim 1 wherein

said aqueous solution consists essentially of 28.0 to 38.0 percent by weight of nitric acid, 8.0 to 20.0 percent by weight of urea and 47.0 to 54.0 percent by weight of water, the molar ratio of urea to nitric acid being 0.15 to 0.6:1.0.

6. The method in accordance with claim 1 wherein said primary metal is selected from the group consisting of tungsten, zirconium, titanium and aluminum, and alloys thereof.

10

**References Cited by the Examiner**

**UNITED STATES PATENTS**

2,177,751 10/1939 Sikorski ----- 156—18 X  
3,192,084 6/1965 Vaughan et al. ----- 156—3

15 ALEXANDER WYMAN, *Primary Examiner*.

JACOB STEINBERG, *Examiner*.